# EUROPEAN PATENT SPECIFICATION

(11) **EP 0 311 203 B1**
(45) Date of publication and mention of the grant of the patent: **22.09.1993**
(21) Application number: 88202172.8
(22) Date of filing: 03.10.1988
(51) Int. Cl.: B22C 1/10

(54) **Foundry core material**
Material für Giessereikerne
Matériau pour noyau de fonderie

(30) Priority: 07.10.1987 GB 8723582
(43) Date of publication of application: 12.04.1989
(73) Proprietor: AE TURBINE COMPONENTS LIMITED, Yeadon Leeds LS19 7AY (GB); THE UNIVERSITY OF LEEDS, Leeds, LS2 9JT (GB)
(72) Inventor: Hamilton, Duncan Havelock, Kirkstall Leeds, LS5 3DL (GB); Roberts, Edward Wilford, Bramhope Leeds (GB)
(74) Representative: Goddard, David John

(56) References cited:
- EP-A- 0 179 649
- GB-A- 829 447
- US-A- 3 002 948
- US-A- 3 661 829

## Description

The present invention relates to ceramic material for use in ceramic cores particularly, though not exclusively for use in the manufacture of precision cast components.

Components such as blades and nozzle guide vanes, for example, for gas turbine engines frequently have complex shaped hollow internal passages for cooling purposes. Such passages allow the component to operate at much high gas inlet temperature than would otherwise be the case. The passages are generally formed by the use of leachable ceramic cores cast in situ during a vacuum precision casting process.

Such cores have generally comprised silica-based materials. The high temperature strength of a core depends on the devitrification of vitreous silica to the crystalline phase, cristobalite. Heretofore this has generally been accomplished by alkali metal ions such as sodium, for example, added to the silica glass as catalysts in minor additions. Although alkali metal ions do promote devitrification of silica they also lower the high temperature strength of the core by lowering the melting temperature of the bond. EP-A-0 179 649 describes silica cores devitrified to cristobalite by the use of alkali metal ions.

In recent years gas turbine components having metallic grain structures comprising either columnar grains, produced by a directional solidification process (DS), or a single crystal (SC) have gained increased prominence. This is due to the higher stresses and temperatures which may be withstood by components having such structures.

Both types of component are made by an essentially similar process wherein any cores used have to withstand temperatures exceeding 1500°C, sometimes for several hours. The result of this may be extensive plastic deformation of the core which tends to deform under its own weight and deflect when metal is poured into the mould in which the core is located.

Outer dimensional tolerances for precision cast gas turbine components are stringent, also the position, size and orientation etc. of cored passages within the components are subject to equally stringent tolerances.

GB-A-82941 is concerned with the production of silica containing ceramics having a crystallised structure. However, the compositions described have of necessity substantial proportions of material other than silica and are manufactured by a process including a melting step which would result in inadequate dimensional accuracy of the resulting cores.

It is an object of the present invention to provide a material for cores which will devitrify without the presence of alkali metal ions and not suffer from distortion at high temperatures.

According to one aspect of the present invention there is provided a core for foundry use, the core comprising silica particles fired together and being at least partially devitrified to cristobalite, the core being characterised by being free of added alkali metal ions and having therein ions selected from the group comprising titanium, zirconium, phosphorus, vanadium, chromium, molybdenum and tungsten.

The ions may be added in the form of a finely divided oxide powder, or as a compound containing the element, preferably an organic compound which is miscible with the binder used during core manufacture. An organic compound miscible with the binder allows homogeneous dispersal throughout the mixture.

Where the element is added as the oxide the addition may lie in the range from 0.05 to 10wt%.

A preferred addition is titania.

A preferred range of titania may be 0.1 to 5wt%.

A more preferred range of titania may be 0.1 to 2.5wt%.

Preferably the silica is of purity greater than 99.5%.

According to a second aspect of the present invention there is provided a method of making a core for foundry use, the method comprising the steps of mixing silica with an organic binder material, moulding a desired core shape, heating to remove the organic binder and then firing characterized in that the mixture prior to firing is free of added alkali metal ions and contains ions selected from the group comprising titanium, zirconium, phosphorus, vanadium, chromium, molybdenum, tungsten and firing is carried out at a temperature in excess of 1180°C such that no melting occurs.

Preferably the firing temperature is in excess of 1200°C.

The content of organic binder material may be in the range of 15 to 40wt% of the mixture.

After firing it is preferred that less than 50% of the silica has transformed to cristobalite, further devitrification continuing during mould preheat so that at casting the cristobalite content approaches 100%.

Titania may be added as titania or as a titanium compound which decomposes to the oxide during processing.

In order that the invention may be more fully understood examples will now be described by way of illustration only.

A series of core material compositions were made by mixing fused silica with 0.1wt%, 0.25wt%, 1.0wt% and 2.5wt% titania of substantially submicron particle size. These compositions were pressed into pellets and fired at temperatures from 1150°C to 1300°C. The extent of devitrification was then assessed by means of thermal expansion measurements. The results showed that titania over the whole range of concentrations tested promoted detrification when fired at and above 1200°C. The extent of crystallisation increased with firing temperature, soak time at temperature and with increasing concentration of titania.

Further material was made of a single composition containing 1wt% titania in the mix to give 1.3wt% in the fired material. The mix comprised 68.50wt% fused silica, 1wt% titania and the balance being an organic binder based on polyethylene glycol. The mix was made in a Z-blade mixer. The organic components were mixed dry with the titania and then the Z-blade mixer was heated until the organic components were molten. Mixing of the molten components and titania was continued for 1 hour and then the silica added in portions. When all the silica had been added mixing continued for 2 hours, the heaters were then switched off and the material granulated in situ. This material was designated mix L69.

A mix was made of a normal production core material containing sodium ions. This material was designated mix 52, and was not in accordance with the present invention.

Test bars of mixes L69 and 52 were injection moulded and heated slowly to a temperature of 700°C to drive off the organic binder materials.

Some of the mix 52 bars were dipped in ethyl silicate solution prior to firing in order to fill some of the porosity in the material. The dipped material was designated A52 and was also not in accordance with the invention.

All three types of material were then fired under similar conditions at 1150°C for 5 hours. Test bars of each of the compositions were then placed from ambient into the hot zone of a Modulus of Rupture (MOR) testing apparatus which had been allowed to stabilise at 1450°C, and soaked for periods of 30 minutes and 60 minutes. After the completion of each soak period the bars were loaded to failure at 55 N/min to failure. After testing physical measurements of porosity and density were made (see Table).

Referring now to the Table and where Mix 52 as fired has a bulk density of 1.45 g/cm³, porosity of 34,1% and a MOR of 7.5 MPa. The effect of dipping in ethyl silicate prior to firing is to increase the bulk density to 1.58 g/cm³ with a decrease in porosity to 28.6% and a consequent doubling of MOR. The L69 bars as fired have a bulk density of 1.43 g/cm³, a porosity of 34.1% and a MOR of 11.0 MPa. The deflection at failure for all compositions is similar at 0.35mm.

It may be seen that the L69 material soaked for 30 and 60 minutes at 1450°C has achieved MOR values of 37.8 and 39.8 MPa. The level of crystallisation of mix 52 and A52 materials is comparable to the L69 material but the MOR values are greatly reduced at averages of 6.8 and 11.8 MPa respectively.

## Claims

1. A core for foundry use, the core comprising silica particles fired together and being at least partially devitrified to cristobalite, the core being characterised by being free of added alkali metal ions and having therein ions selected from the group comprising titanium, zirconium, phosphorus, vanadium, chromium, molybdenum and tungsten.

2. A core according to claim 1 characterised in that the ions are present in the form of an oxide.

3. A core according to claim 2 characterised in that the oxide content is titania.

4. A core according to claim 2 or claim 3 characterised in that the oxide content is from 0.05 to 10.0 wt%.

5. A core according to claim 4 characterised in that the oxide content is from 0.1 to 5.0 wt%.

6. A core according to claim 4 characterised in that the oxide content is from 0.1 to 2.5 wt%.

7. A method of making a core for foundry use, the method comprising the steps of mixing silica with an organic binder material, moulding a desired core shape, heating to remove the organic binder and then firing characterized in that the mixture prior to firing is free of added alkali metal ions and contains ions selected from the group comprising titanium, zirconium, phosphorus, vanadium, chromium, molybdenum, tungsten and firing is carried out at a temperature in excess of 1180°C such that no melting occurs.

8. A method according to claim 7 characterised in that after firing the core is further heated in a mould during pre heating of the mould prior to casting of metal into the mould.

9. A method according to claim 8 characterized in that the core is held for up to 60 minutes at the mould preheat temperature.

10. A method according to claim 9 characterized in that the mould preheat temperature is about 1450°C.

11. A method according to any one of preceeding claims 7 to 10 characterised in that the firing temperature is in excess of 1200°C.

12. A method according to claim 11 characterized in that the firing temperature lies in the range from 1200°C to 1300°C.

13. A method according to any one preceeding claim from 7 to 12 characterized in that the ions are added in the form of a finely divided oxide.

14. A method according to any one preceeding claim from 7 to 12 characterized in that the ions are added as an organic compound.

15. A method according to claim 14 characterized in that the organic compound is miscible with the organic binder material.

16. A method according to claim 13 characterized in that the oxide is titania.

17. A method according to claim 16 characterised in that the titania content of the mixture is from 0.05 to 10.0 wt%.

18. A method according to claim 17 characterized in that the titania content of the mixture is from 0.1 to 5.0 wt%.

19. A method according to claim 17 characterized in that the titania content of the mixture is from 0.1 to 2.5 wt%.

## Patentansprüche

1. Gießereikern, der Siliziumdioxid-Partikel, die zusammengebrannt sind, aufweist und zumindest teilweise zu Cristobalit entglast wurde, **dadurch gekennzeichnet**, daß er frei von Zugaben von Alkalimetall-Ionen ist und Ionen aufweist, die aus der Gruppe ausgewählt sind, welche Titan, Zirkonium, Phosphor, Vanadium, Chrom, Molybdän und Kupfer umfaßt.

2. Gießereikern nach Anspruch 1, dadurch gekennzeichnet, daß die Ionen in Form eines Oxids vorliegen.

3. Gießereikern nach Anspruch 2, dadurch gekennzeichnet, daß der Oxidgehalt Titandioxid ist.

4. Gießereikern nach Anspruch 2 oder Anspruch 3, dadurch gekennzeichnet, daß der Oxidgehalt von 0,05 bis 10 Gew.-% beträgt.

5. Gießereikern nach Anspruch 4, dadurch gekennzeichnet, daß der Oxidgehalt von 0,1 bis 5,0 Gew.-% beträgt.

6. Gießereikern nach Anspruch 4, dadurch gekennzeichnet, daß der Oxidgehalt von 0,1 bis 2,5 Gew.-% beträgt.

7. Verfahren zur Herstellung eines Gießereikernes, das die Schritte Mischen von Siliziumdioxid mit einem organischen Bindemittel, Formen einer gewünschten Kernform, Erhitzen zum Entfernen des organischen Bindemittels und anschließendes Brennen aufweist, dadurch gekennzeichnet, daß die Mischung vor dem Brennen frei von Alkalimetallionen-Zugaben ist und Ionen enthält, die ausgewählt sind aus der Gruppe, welche Titan, Zirkonium, Phosphor, Vanadium, Chrom, Molybdän und Kupfer umfaßt, und daß das Brennen bei einer Temperatur über 1180°C so vorgenommen wird, daß kein Schmelzen auftritt.

8. Verfahren nach Anspruch 7, dadurch gekennzeichnet, daß der Kern nach dem Brennen noch weiter in einer Form während deren Vorheizens vor dem Vergießen des Metalls in diese erhitzt wird.

9. Verfahren nach Anspruch 8, dadurch gekennzeichnet, daß der Kern bis zu 60 min auf der Form-Vorheiztemperatur gehalten wird.

10. Verfahren nach Anspruch 9, dadurch gekennzeichnet, daß die Form-Vorheiztemperatur etwa 1450°C beträgt.

11. Verfahren nach einem der vorhergehenden Ansprüche 7 bis 10, dadurch gekennzeichnet, daß die Brenntemperatur oberhalb 1200°C liegt.

12. Verfahren nach Anspruch 11, dadurch gekennzeichnet, daß die Brenntemperatur im Bereich von 1200°C bis 1300°C liegt.

13. Verfahren nach einem der vorhergehenden Ansprüche 7 bis 12, dadurch gekennzeichnet, daß die Ionen in Form eines feinzerteilten Oxids zugegeben werden.

14. Verfahren nach einem der vorhergehenden Ansprüche 7 bis 12, dadurch gekennzeichnet, daß die Ionen in Form einer organischen Verbindung zugegeben werden.

15. Verfahren nach Anspruch 14, dadurch gekennzeichnet, daß die organische Verbindung mit dem Material des organischen Bindemittels mischbar ist.

16. Verfahren nach Anspruch 13, dadurch gekennzeichnet, daß das Oxid Titandioxid ist.

17. Verfahren nach Anspruch 16, dadurch gekennzeichnet, daß der Titandioxidgehalt der Mischung von 0,05 bis 10,0 Gew.-% beträgt.

18. Verfahren nach Anspruch 17, dadurch gekennzeichnet, daß der Titandioxidgehalt der Mischung von 0,1 bis 5,0 Gew.-% beträgt.

19. Verfahren nach Anspruch 17, dadurch gekennzeichnet, daß der Titandioxidgehalt der Mischung von 0,1 bis 2,5 Gew.-% beträgt.

## Revendications

1. Noyau pour fonderie, le noyau comprenant des particules de silice chauffées ensembles et étant au moins partiellement dévitrifiées en cristobalite, le noyau étant caractérisé en ce qu'il est libre de tout ion métallique alcalin ajouté et en ce qu'il comporte des ions choisis parmi le groupe comprenant du titane, zirconium, phosphore, vanadium, chrome, molybdène et tungstène.

2. Noyau selon la revendication 1, caractérisée en ce que les ions se présentent sous la forme d'un oxyde.

3. Noyau selon la revendication 2, caractérisé en ce que le contenu de l'oxyde est de l'oxyde de titane.

4. Noyau selon la revendication 2 ou la revendication 3, caractérisé en ce que la teneur en oxyde est comprise entre 0,05 et 10,0 % en poids.

5. Noyau selon la revendication 4 caractérisé en ce que la teneur en oxyde est compris entre 0,1 et 5,0 % en poids.

6. Noyau selon la revendication 5 caractérisé en ce que la teneur en oxyde est comprise entre 0,1 et 2,5 % en poids.

7. Méthode pour réaliser un noyau de fonderie, la méthode comprenant les étapes de : mélanger de la silice avec un matériau liant organique, mouler un noyau selon une forme donnée, chauffer pour enlever le liant organique et ensuite cuire, caractérisée en ce que le mélange, avant la cuisson, est libre d'ions métalliques alcalins ajoutés, et contient des ions choisis parmi le groupe comprenant du titane, zirconium, phosphore, vanadium, chrome, molybdène, tungstène, et la cuisson est réalisée à une température supérieure à 1180°C de façon qu'aucune fusion n'apparaisse.

8. Méthode selon la revendication 7, caractérisée en ce que, après la cuisson, le noyau est ensuite chauffé dans un moule pendant le pré-chauffage du moule avant la coulée de métal dans le moule.

9. Méthode selon la revendication 8, caractérisée en ce que le noyau est maintenu jusqu'à 60 minutes à la température de pré-chauffage du moule.

10. Méthode selon la revendication 9, caractérisée en ce que la température du pré-chauffage du moule est d'environ 1450°C.

11. Méthode selon l'une des revendications précédentes 7 à 10, caractérisées en ce que la température de cuisson est supérieure à 1200°C.

12. Méthode selon la revendication 11, caractérisée en ce que la température de cuisson est comprise entre 1200°C et 1300°C.

13. Méthode selon l'une des revendications précédentes 7 à 12, caractérisée en ce que les ions sont ajoutés sous la forme d'un oxyde finement divisé.

14. Méthode selon l'une des revendications précédentes 7 à 12, caractérisée en ce que les ions sont ajoutés sous forme d'un composé organique.

15. Méthode selon la revendication 14, caractérisée en ce que le composé organique est miscible avec le matériau liant organique.

16. Méthode selon la revendication 13, caractérisée en ce que l'oxyde est de l'oxyde de titane.

17. Méthode selon la revendication 16, caractérisée en ce que la teneur en oxyde de titane du mélange est comprise entre 0,05 et 10,0 % en poids.

18. Méthode selon la revendication 17, caractérisée en ce que la teneur en oxyde de titane du mélange est comprise entre 0,1 et 5,0 % en poids.

19. Méthode selon la revendication 17, caractérisée en ce que la teneur en oxyde de titane du mélange est comprise entre 0,1 et 2,5 % en poids.
